

## UNITED STATES PATENT OFFICE

CARL NITTINGER, OF BRESLAU, GERMANY, ASSIGNOR TO CARNITT-ROSTSCHUTZ & FARBSTOFF G. M. B. H., OF BRESLAU, GERMANY

## PROCESS OF PRODUCING BRIGHT PAINTS

No Drawing. Application filed October 31, 1927, Serial No. 230,166, and in Germany May 14, 1927.

This invention relates to a process of producing paints for iron, wood and the like possessing metallic brightness and consisting of ground coal slag and a binding matter.

- 5 The characteristic feature of the invention consists in that to the ground slag electro-positive zinc powder is added prior to admixing the slag with the binding matter. It has been proposed, to use electropositive zinc as 10 rust preventing means, but the durability of a paint with zinc is very limited as the zinc with the binding matter does not enter into an intimate combination with the iron or wood. When, however, according to the new 15 process, ground coal slag is admixed with finely ground electropositive zinc and, with the addition of a binding matter, is used as paint, the zinc increases the rust-preventing capability of the coal slag and goes, together 20 with the coal slag, into an intimate combination with the iron, wood or the like, so that such a paint is a much better rust protection than all the commonly used rust preventing paints and the durability of the paint becomes 25 illimitable. The zinc, in the combination of electropositive zinc with the coal slag, obtains the softness which the coal slag in combination with its binding matter possesses, so that the paint can not longer scale off 30 the painted body, even when this body is submitted to alterations of shape.

For carrying out the process about 80% of finely ground coal slag are mixed with about 20% of finely ground electropositive 35 zinc and to this mixture the desired quantity of binding matter, varnish or the like, is added.

The painting might be carried out also by 40 painting the surface with varnish and in blowing onto this coating of varnish the mixture of coal slag and electropositive zinc. The colour tone of the ground slag can be altered by addition of mixed colours, and the mass may be used as spattle-cement.

45 The term "coal slag" as used herein is intended to refer to that product which results where coal is burned at very high temperatures and where the melting point of the ashes is passed. The slag or molten ashes 50 generally comprise silicates or glasses and

the improved results of the invention are attributed to the fact that the powdered coal slag used as a pigment contains just the amount of molten impurities (unburned coal, i. e. coke, iron in the form of pyrite, and other 55 minerals) which are desired to give the desired excellent results.

I claim:—

1. A rust resisting paint comprising about eighty percent of finely ground coal slag, 60 about twenty percent of finely ground electro-positive zinc, and a vehicle.
2. An iron article having a coating containing finely ground coal slag and finely ground electro-positive zinc. 65

In testimony whereof I affix my signature.

CARL NITTINGER.

70

75

80

85

90

95

100